

No. 851,684.

PATENTED APR. 30, 1907.

J. F. MONNOT.

PROCESS OF MAKING COMPOUND METAL BODIES.

APPLICATION FILED JUNE 16, 1905. RENEWED AUG. 21, 1906.



Attest:

Comitchell  
a. L. O'Brien

Inventor:

JOHN FERREOL MONNOT  
by Dickenson, Brown, Rægener & Birney  
Atty's.

# UNITED STATES PATENT OFFICE.

JOHN FERREOL MONNOT, OF NEW YORK, N. Y.

## PROCESS OF MAKING COMPOUND METAL BODIES.

No. 851,684.

Specification of Letters Patent.

Patented April 30, 1907.

Application filed June 16, 1905. Renewed August 21, 1906. Serial No. 331,522.

*To all whom it may concern:*

Be it known that I, JOHN FERREOL MONNOT, a citizen of the United States, and a resident of the borough of Manhattan, city, county, and State of New York, have invented 5 certain new and useful Improvements in Processes of Making Compound Metal Bodies, of which the following is a specification, accompanied by drawings.

My invention relates to improvements in processes of making compound metal bodies, such articles comprising ingots, plates, sheets, rods, tubes, wire, structural shapes and other articles composed of layers or 15 strata of unlike metals firmly and autogenously welded together.

My novel invention consists in the novel process herein described for producing such articles; all as more fully hereinafter set 20 forth, matters of novelty being particularly pointed out in the appended claims.

Compound articles composed of unlike metals welded together may be used to great advantage in a variety of arts and for many 25 different purposes, as combining the specific advantages of the component metals. For example, plates, sheets, etc., composed of a strong but readily oxidizable metal such as iron or steel, covered with an impervious co- 30 herent coating of copper or other less oxidizable metal, may be used to great advantage in lieu of ordinary iron or steel plates, sheets, etc., wherever such articles are to be exposed to the weather, air or other oxidizing influences, or to the action of corroding liquids, 35 gases or vapors which readily attack iron or steel but do not attack at all, or at least to so serious an extent, the coating metal employed. Such articles composed of copper, 40 brass, silver, aluminium, etc., backed with iron or steel may be used with great advantage where considerable strength or stiffness of metal is desired, coupled with the chemical, physical, electrical or other properties 45 or color or appearance of the non-ferrous metals mentioned. For electrical conductors it is desirable to combine the high electrical conductivity of copper, aluminium, etc., with the great strength of steel. Many 50 other such uses might be pointed out. In all such cases, it is a prime requisite that the unlike metals shall be so inseparably united that a compound ingot formed by joining them shall be capable of great extension or 55 working, as by rolling, drawing, etc., to make thin sheets, rods, angles, tubes, wire, etc.,

without separation of the united layers, without development of seams, pores, flaws, etc.; and it is in practice desirable that during such working, the strata of the joined metals 60 shall maintain substantially their original relative proportions, even down to the thinness extended article produced.

The object of my present invention is to devise a method of making such compound 65 ingots from such pairs of unlike metals as steel and copper, steel and brass or other copper alloys, steel and silver, steel and aluminium, nickel and copper, or indeed any other pair of substantially unlike metals 70 that is, metals or alloys of unlike chemical nature; to form such bimetallic ingots of any desired shape or dimensions and with any desired relative proportions of the component 75 metals; to produce such a strong, autogenous and weld-like union between such unlike metals as shall be incapable of separation by heat or mechanical stress and shall be adapted to permit indefinite coextension of the joined metals in a compound ingot by any of 80 the ordinary methods of working with said union extending throughout and persisting at all meeting points of the joined metals, and with the same relative proportions of the component unlike metals in the extended 85 ware as in the original compound ingot; to produce in such coextended ware articles which shall be comparable in price with ordinary coated metals, like electroplated, tinned and galvanized ware while far superior 90 in quality; to produce in such coated ware, coatings which shall be hard, dense, free from all pores, scale spots, flaws, blisters or points of separation and shall be welded 95 united with the base metal throughout; and it is, further, my object in said method to accomplish these desirable ends by a simple, cheap and easy process requiring no highly skilled labor.

Suitable apparatus for carrying out my 100 process is shown in the accompanying drawings in which:—

Figure 1 shows a vertical section of suitable apparatus, showing the parts in one position, and Fig. 2 is an elevation, partly in 105 section, showing the parts in a different position.

Briefly stated, the process in my present invention consists in thoroughly cleaning a 110 base or core of the more infusible metal; bringing it up to a welding temperature without permitting access of air and consequent

oxidation during heating; contacting with it on the cleaned surfaces a highly-heated, or "supermolten", mass of a molten unlike metal; segregating from said mass in immediate proximity to the base a layer of the thickness desired in the subsequent compound ingot; allowing base and coating layer to cool under or during compression; and extending the compound ingot so formed to produce the extended ware desired. It is obvious that many ways of performing this broad process may be devised, and I shall hereinafter describe one such which may be used. For the sake of simplicity, I shall in the main describe the production of a compound steel-copper ingot, it being understood that this is typical, within the limits of my broad invention, of the manner of making compound ingots of the other pairs of unlike metals.

The steel core or base used may be an ingot, bar, bloom, billet or other commercial form, and may be of any desired cross-section, as round, square, oval, etc., and of any size. It is to be cleaned in any of the ordinary well-understood ways, care only being taken during the cleansing to insure the complete removal of scale, oxid, dirt or other foreign matter which might later interfere with the absolute contact of the metal with the unlike metal. A clean metallic surface should be obtained.

Heating may be done in any desired way, provided that care be taken to prevent oxidation or other contamination of the cleaned metal. It is highly desirable that air should not gain access to the clean surfaces while they are hot. The heating may be done by the heat of the bath of the molten unlike metal used for coating, or separately performed. I ordinarily prefer the latter as avoiding delay in the coating operation proper where a rapid succession of bases are to be coated, large baths of highly heated coating metal such as copper, being difficult to handle, expensive and subject to rapid oxidation, which renders it undesirable to prolong the period of immersion or contact of the base to be coated. I therefore frequently employ a separate preliminary heating bath of molten fluxes or indifferent salts in which or by which the steel core may be heated to the necessary degree without opportunity for contamination or oxidation of the clean metallic surfaces. For this bath any fusible salt or flux not attacking the metal may be used, such as borax, sodium chlorid, sodium carbonate, fluor-spar, etc., and the core may be heated therein until it reaches the proper temperature for contacting with the subsequent bath of highly heated molten copper. It should be heated to or near the welding temperature, and, in cases where the ingot is to be directly worked after coating, sufficiently long to allow permeation

of heat throughout. In removing the heated core from the bath of molten flux, a coating of the latter will be found to adhere and shield the metal from access of air while in transit to the bath of molten copper. In contacting with the latter, the flux will flow away or slag off, before the copper as the latter, so to speak, "wets" the steel, thereby insuring that absolute metallic surfaces of the two metals shall contact without opportunity for access of air. For this flux bath in welding copper to steel, I may use fluor-spar. This substance melts at about 950 degrees centigrade, or somewhat below the melting point of copper, 1050 degrees, and a steel core immersed in or contacted with a bath of molten fluor-spar readily attains the necessary degree and amount of heat. With coating metals of lower melting point than copper, such as aluminium, it may be preferable to use another flux. But of course where in practice it may be deemed desirable, the preliminary flux bath may be omitted and the clean core plunged directly into or contacted with the highly heated molten copper, which will soon bring it up to the desired temperature. Other methods of heating are described in my copending application, Serial # 261,739, filed May 23, 1905. Whichever way of heating is adopted, the steel core is heated to a welding temperature, or a temperature at which it exhibits a measure of molecular activity, and upon the subsequent contact with the highly heated molten copper, a superficial alloy coating or film is formed, upon which the main mass of copper readily welds.

Referring to the drawings, A represents a large crucible of any suitable character which may be filled with a mass or bath, B, of highly heated molten copper or suitable metal to be used for coating the compound ingot to be formed. Core or base, C, is of an unlike, more infusible metal, in this instance assumed to be steel, and may be an ingot, billet, slab or bar of round, square, oval or other shape. Means are shown for handling this core or base, in this instance the means being a rod D which may be temporarily connected to the core and is suitably suspended, as by means of the hook E, which may be raised or lowered by any suitable means, here shown as a compressed air lift, F. A guide G slides over the rod D and is also arranged to be raised and lowered by means of air lifts, as shown, rods H being adapted to connect guide and lifts. The piston of the main cylinder carries a cross-head on which are mounted the auxiliary cylinders which actuate the guide G, carrying the casing I which may therefore be raised and lowered out of or into the bath B of molten metal. In this instance a suitable chuck, J, is shown carried by the guide G for supporting casing I. As shown, there is secured to the lower end of the billet or

core, a plate or bottom flange K, provided with a groove L adapted to receive the lower edge, O, of the jacketing casing I when at its lowermost position, as shown in Fig. 2. The 5 relative diameters of the core C and casing I are such that the interval between their sides, as indicated in Fig. 2, corresponds to the thickness of coating metal to be placed on core C.

10 In using the described apparatus to carry out my process, a suitably cleaned core, previously heated if desired, may be secured to the handling rod D, and the bottom plate or flange, K, secured to its base. The core is then lowered into the bath B, of molten copper or other suitable metal, preferably completely submerging it. This coating metal is maintained in a molten, highly heated condition by any suitable heating means, as a 15 furnace (not shown). When the core has reached substantially the temperature of the molten metal, which takes but a few minutes, the mold or casing I is lowered around core C until its lower edge, O, enters the groove L of the bottom plate or flange, K. Core and casing are kept spaced apart to the proper distance by the guide G and by the coöperating groove and edge in bottom plate and casing, respectively. This distance is 20 such as to form or segregate a layer of the molten metal of the thickness of the coating desired to appear on the resultant compound ingot. Segregation is done by the lowering of the casing I. As soon as casing I and bottom plate K come together, the casing is 25 quickly lifted out of the molten metal bath by means of the air lift, carrying with it the contained core and the segregated layer of molten metal surrounding it, and is allowed 30 to cool sufficiently to set said layer of coating metal firmly on the core. The whole operation is preferably conducted as quickly as possible. The compound ingot so formed may then be removed from the casing or 35 mold, and, in cases where the initial heat applied has been sufficient to permeate the entire core, will be found still hot enough to permit direct rolling or other working. This 40 immediate rolling, etc., has the double advantage of saving a reheating and of perfecting the weld of the two metals, suppressing small flaws or porosity which may exist or be formed in the coating metal.

45 In setting, the coating layer will cool more rapidly than the core metal, and as the coefficient of expansion and contraction is generally greater in coating metals like copper, silver, etc., than in those used for cores, such as steel, in such an annular coated ingot as 50 is made by the apparatus and in the procedure just described, the natural contraction of the coating metal will produce enough compression to complete the weld upon the meeting surfaces of the two unlike metals.

55 In fact the pressure so obtained is often so

great as to produce damaging strains, cracks, etc., in the coating if the compound ingot be allowed to cool entirely. And although I have produced a perfect weld of two unlike metals in this manner without the use of extraneous pressure, I usually prefer to work the ingot while hot. In some cases, I may complete and perfect the weld by applying pressure on the compound ingot after the immersion and when at a suitable temperature, either by means of a hydraulic press or by other suitable mechanical means. 70

In making compound ingots with a non-annular coating, extraneous pressure is usually necessary, for the reasons specified, 80 although by contacting the perfectly clean base with molten unlike metal of a suitably high temperature I produce a superficial alloy coating or film of the two metals on which the coating will weld without pressure. 85

The apparatus shown and the procedure described are to be understood as representing merely convenient and practical means for carrying out my process. The procedure may be varied within the limits of my broad disclosure and many specific forms of apparatus may be devised suitable for my purpose. The particular type of apparatus used is not material to the successful carrying out of my process. 90

95 What I claim and desire to secure by Letters Patent of the United States is:—

1. The process of producing compound metal bodies of unlike metals autogenously welded together which consists in contacting with a base of one such metal a highly heated molten mass of another and unlike metal, segregating from such molten mass the layer thereof of molten metal in immediate proximity to and in contact with said base and allowing it to set thereagainst. 105

2. The process of producing compound metal bodies comprising steel and an unlike metal autogenously welded together which consists in contacting with a steel base a highly heated molten mass of an unlike metal, segregating from such molten mass the layer of molten metal in immediate proximity to and in contact with said steel base, and allowing it to set thereagainst. 110

3. The process of producing compound metal bodies comprising steel and copper autogenously welded together which consists in contacting with a steel base a highly heated molten mass of copper, segregating from such molten mass of copper the layer of molten metal in immediate proximity to and in contact with said steel base and allowing it to set thereagainst. 115

4. The process of producing coextended compound metal ware composed of unlike metals autogenously welded together which consists in contacting with a base of one such metal a highly heated molten mass of another and unlike metal, segregating from 120

130

- such molten mass the layer of molten metal in immediate proximity to and contact with said base, allowing it to set thereagainst, and extending the compound ingot so formed while in a heated condition.
5. The process of producing compound metal bodies of unlike metals autogenously welded together, which consists in immersing a base of one such metal in a highly heated molten bath of another and unlike metal, segregating from said bath the layer of said molten metal surrounding said base and allowing it to set thereagainst.
15. The process of producing compound metal bodies comprising steel and an unlike metal autogenously welded together, which consists in immersing a base of steel in a highly heated molten bath of such unlike metal, segregating from said bath the layer 20 of said molten metal surrounding the base, and allowing it to set thereagainst.
25. The process of producing compound metal bodies comprising steel and copper autogenously welded together which consists in immersing a base of steel in a highly heated molten bath of copper, segregating from said bath the layer of molten copper surrounding the base, and allowing it to set thereagainst.
30. 8. The process of producing compound metal bodies of unlike metals autogenously welded together which consists in immersing a hot clean base of one such metal in a highly heated molten mass of another and unlike 35 metal, segregating the layer of said molten metal in contact with said base, withdrawing base and contacting layer and allowing said layer to set against said base.
40. 9. The process of producing compound metal bodies comprising steel and an unlike metal autogenously welded together which consists in immersing a hot clean steel base in a highly heated molten mass of another and unlike metal, segregating the layer of 45 said molten metal in contact with said base, withdrawing base and contacting layer, and allowing said layer to set against said base.
50. 10. The process of producing compound metal bodies comprising steel and copper autogenously welded together which consists in immersing a hot clean steel base in a highly heated molten mass of copper, segregating the layer of said molten copper in contact with said base, withdrawing base and 55 contacting layer, and allowing said layer to set against said base.
60. 11. The process of producing coextending compound metal ware composed of unlike metals autogenously welded together which consists in immersing a hot clean base of one such metal in a highly heated molten bath of another and unlike metal, segregating the layer of said molten metal in contact with said base, withdrawing base and contacting 65 layer, allowing the layer to set against the base, and coextending the compound ingot formed while still hot.
12. The process substantially as hereinafter described of making bi-metallic products, such as ingots, sheets, tubes, wires and the like, of different metals welded together which consists in heating a core of the desired metal to a welding temperature in a bath of molten metal for the coating of a different kind from the core, to produce a superficial alloy of the core metal and coating metal out of the action of the air, thereby insuring a perfect weld, segregating a layer of molten metal from said bath in contact with said core, removing the core and its coating from the bath, and then working the sufficiently cooled bi-metallic ingot in a rolling mill or other suitable mill to produce bi-metallic plates, sheets, tubes, wires and like products.
70. 13. The process substantially as hereinafter described of making bi-metallic products, such as ingots, sheets, tubes, wires and the like, of different metals welded together which consists in first cleaning the surface of a core of the desired metal, heating said core 75 preliminarily to a suitable temperature in such manner as to prevent oxidation, immersing the core in a bath of molten metal for the coating of a different kind from the core thereby completing the heating of the 80 core and bringing it to a welding temperature, separating a layer of the molten metal from the bath of the desired thickness for the coating, removing the core and its coating from the bath and working the bi-metallic ingot in a rolling mill or other suitable mill to produce 85 bi-metallic plates, sheets, tubes, wires and like products.
90. 14. The process substantially as hereinafter described, of making compound metal products of different metals welded together which consists in immersing a core of the desired metal in a bath of molten metal for the coating of a different kind from the core, thereby heating the core to a welding temperature, separating a layer of the molten metal from the bath of the desired thickness for the coating, removing the core and its coating from the bath, and permitting the coating to solidify upon said core.
95. 15. The process substantially as hereinafter described of making bi-metallic products, such as ingots, sheets, tubes, wires and the like, of different metals welded together which consists in heating a core of the desired metal to a temperature near the melting point of the coating metal in such manner as to prevent oxidation, immersing the core in a bath of molten metal for the coating of a different kind from the core, thereby completing the heating of the core and bringing it to a welding temperature, segregating a layer of molten metal from said bath in contact with said core and then working the sufficiently cooled bi-metallic ingot in a rolling mill or 100
105. 115. 120. 125. 130.

other suitable mill, to produce bi-metallic sheets, tubes, wires, and like products.

16. The process substantially as hereinafter described of making compound metal products of different metals welded together which consists in surrounding a core of the desired metal with a bath of molten metal for the coating of a different kind from the core thereby heating the core to a welding temperature, separating a layer of the molten metal around the core from the remainder of the bath of the desired thickness for the coating, removing the core and its coating from the bath and permitting the coating to solidify upon said core.

17. The process substantially as hereinafter described of making bi-metallic products, such as ingots, sheets, tubes, wires and the like of different metals welded together which consists in heating the core to a high temperature in a bath of molten metal for the coating of a different kind from the core, to produce a superficial alloy of the core metal and coating metal, thereby insuring a perfect weld, then separating a layer of the molten metal from the bath of the desired thickness for the coating and removing the core and its coating from the bath.

18. The process substantially as hereinafter described of making bi-metallic products, such as ingots, sheets, tubes, wires and the like of different metals welded together which consists in heating the core to a high temperature in a bath of molten metal for the coating of a different kind from the core, to produce a superficial alloy of the core metal and

coating metal, thereby insuring a perfect weld, then separating a layer of the molten metal from the bath of the desired thickness for the coating and removing the core and its coating from the bath, then forcing the core and the coating metal together by pressure applied to the entire surface of contact of the metals while at a suitable temperature to perfect the weld and suppress any flaws in the coating metal, and finally working the bi-metallic ingot in a rolling mill or other suitable mill to produce bi-metallic plates, sheets, tubes, wires, and like products.

19. The process substantially as hereinafter described of making bi-metallic products, such as ingots, sheets, tubes, wires and the like, of different metals welded together which consists in first heating the core in a bath of a molten metal, having a lower melting point than the coating metal, then immersing the core thus heated in a bath of molten coating metal of a different kind from the core to finish heating the core and bring it to welding temperature, separating a layer of the molten metal around the core from the remainder of the bath of the desired thickness for the coating, and finally removing the core and its coating from the bath.

In testimony whereof I have signed this specification in the presence of two subscribing witnesses.

JOHN FERREOL MONNOT.

Witnesses:

A. L. O'BRIEN,  
E. P. LA SAY.